

April 3, 1934.

R. E. REED

1,953,898

PLASTER OF PARIS BANDAGE AND METHOD OF PREPARING SAME

Filed March 13, 1931

Fig-1



Fig-2



Inventor  
Raymond E. Reed,  
By: Carl S. Blay

Atty.

## UNITED STATES PATENT OFFICE

1,953,898

PLASTER OF PARIS BANDAGE AND METHOD  
OF PREPARING SAMERaymond E. Reed, Chicago, Ill., assignor to The  
Kendall Company, Chicago, Ill., a corporation  
of Massachusetts

Application March 13, 1931, Serial No. 522,494

5 Claims. (Cl. 128—91)

This invention relates to a plaster of Paris bandage adapted for use in making surgical casts, and to a method of preparing the same for shipment and handling.

5 Bandages of the type referred to are ordinarily made by spreading the plaster in powdered or finely divided condition over strips of loosely woven fabric, such as gauze or crinoline, which are then wound into rolls of size suitable for casting purposes. In some cases the plaster, instead of being applied to the gauze in dry condition, is applied in the form of a thin paste which, when dried, leaves the plaster in the form of a more or less continuous crust or coating. This type, 10 however, is inconvenient to handle in the making of the cast, because of the tendency for the coils of the roll to telescope and become tangled when the roll is immersed in water preparatory to making the cast. Also the bandages which contain the plaster in finely divided condition are 15 very messy. When the roll is removed from the carton by the physician, loose plaster is likely to fall over his hands.

20 The object of my invention is to provide a plaster of Paris bandage consisting of a neat, dust-proof unit which may be easily handled by the physician without danger of losing any considerable part of the plaster in applying the bandage and without encountering the trouble caused by 25 unwinding and telescoping of the coils thereof; also to provide a novel method of producing such a bandage.

25 The invention will be understood from the following detailed description, which, taken in connection with the accompanying drawing, discloses 30 a preferred embodiment thereof.

Referring to the drawing:

Fig. 1 is a perspective view of a surgical bandage constructed according to my invention, an 35 outer portion of the bandage being broken away 40 to show the internal structure; and

Fig. 2 is a view of the bandage taken as indicated by line 2—2 of Fig. 1.

Generally stated, the invention resides in 45 the provision of a thin protective coating on the surfaces of the ordinary rolled plaster of Paris bandage. The coating comprises material which has sufficient adhesive properties to hold the rolled unit in wound-up condition and which is 50 easily penetrated by water when the bandage is dipped preparatory to use.

In the drawing, numeral 3 designates generally an ordinary form of rolled plaster of Paris bandage consisting of a series of fabric coils 4 55 containing plaster either in powdered form or in the form of an encrusting coating. In the ordinary form in which rolls of this type are marketed the fabric may be unwound while the bandage is in the dry condition, the entire put-up 60 being more or less loose, so that care must be

taken in dipping the bandage to prevent telescoping of the coils. The protective coating which is applied to a roll of this type, in accordance with my invention, is indicated by the numeral 5, and is present in the form of a thin layer which 65 covers both the end surfaces of the roll as well as the inner and outer cylindrical side walls.

The coating 5 is preferably applied by dipping the rolled bandage in a solution of a material which, when dried, will be easily penetrated by 70 water, and which in the dry condition will have sufficient adhesive properties to hold the coils together as a compact dust-proof unit. The solution of the adhesive material into which the 75 rolled bandages are dipped, also preferably contains plaster of Paris in an amount sufficient to give the solution the consistency of a thin paste.

The following is an example of a preferred composition for the dipping solution:

|                      | Pounds |
|----------------------|--------|
| Gelatine (agar-agar) | 80     |
| Ammonium acetate     | 5 1/2  |
| Plaster of Paris     | 6      |
| Water                | 105    |
|                      | 220    |

The gelatine is added to the water and heated to 85 boiling, and the solution is then cooled. The ammonium acetate is then dissolved in the solution, after which the plaster in powdered form is introduced with thorough stirring. This solution has the consistency of a thin paste. The 90 coating 5 is applied by dipping the rolled bandages in this solution and then drying.

The gelatine in the above formula constitutes 95 the adhesive material which holds together the plaster in the dried coating to form a tough non-chipping protective surface. It is not necessary, however, to use plaster of Paris in the above formula inasmuch as the gelatine alone will form an adhesive coating. When omitting plaster of 100 Paris from the solution, the procedure is substantially the same as above outlined, the bandages being dipped in the solution of gelatine and ammonium acetate, and then dried.

The ammonium acetate serves as a retardant 105 to prevent premature hardening of the plaster. Even though no plaster is used in the dipping solution, a retardant is desirable to prevent premature hardening of the plaster on the outer surfaces of the roll which are moistened when the bandage is dipped. The ammonium acetate, 110 being volatile, is not present in the final coating, it being driven off with the water in the drying operation.

A firm and satisfactory adhesive coating may 115 be provided without following strictly the above-outlined preferred procedure. For example, it is not necessary that the solution of gelatine be first boiled before incorporating the retardant and before adding the plaster. Also, it is not necessary to use a retardant. However, when 120

the retardent is omitted, it is necessary to work the process at a temperature of 98° centigrade, or higher, to prevent premature hardening. As an example of this latter procedure, the following is given:

The rolled bandages are preliminarily heated to a temperature of about 98° centigrade, and are then dipped in a boiling solution comprising the following mixture:

|                  | Pounds |
|------------------|--------|
| Gum arabic       | 2      |
| Plaster of Paris | 50     |
| Water            | 100    |

15 The dipped bandages are dried at a temperature not lower than 98° centigrade.

16 The coating obtained by following any one of the above outlined procedures will bind together the coils of the roll to prevent falling of loose plaster from the bandage. If plaster is used in the dipping solution, a somewhat heavier coating is formed than will be formed by the adhesive material alone. Either type of coating, however, will effectively prevent loss of plaster and uncoiling of the roll when it is being made ready for use.

17 Various adhesive materials in addition to the gelatine and gum arabic, indicated in the above examples, may be used, among which may be mentioned sugar, dextrine, starch, and various water-soluble gums, such as gum ghatti. Also various ammonium salts such as ammonium carbonate, ammonium bicarbonate, ammonium hypophosphate, ammonium chloride, and ammonium citrate, may be used as retardents in lieu of the ammonium acetate in the above examples.

18 The invention provides a plaster bandage which is exceedingly convenient to handle, and which also is not likely to be affected by moisture in the air, by reason of the protection afforded by the outer protective covering. The method of treatment is easily carried out and requires only the use of materials which are comparatively cheap. The dried coating is very thin and is easily penetrated by water when the roll is immersed, thereby avoiding any delay or inconvenience in handling when the bandage is being made ready for casting purposes.

19 While said coating is water-permeable, however, it does not readily break down even after immersion in water, and therefore prevents an excess of water from entering between the layers of the roll, thus making it unnecessary to squeeze or wring out the roll after immersion, as is necessary with the ordinary plaster of Paris bandage. Great difficulty has heretofore been experienced by reason of the fact that upon immersion the roll becomes super-saturated and is likely to telescope in the hands of the surgeon due to the fact that the plaster-coated layers are rendered slippery and unruly for handling. In addition to the danger of telescoping, the usual form of bandage becomes very messy in the process of removing the excess water, thus making it extremely difficult to apply the bandage. Both these difficulties are overcome by my invention since the coating, while sufficiently permeable to permit enough water to enter the roll to moisten the plaster, does not disintegrate upon immersion, and therefore prevents an excess of water from entering between the layers of the roll, thus avoiding any necessity for wringing out the roll and preventing telescoping of the latter.

20 The foregoing detailed description has been

given for clearness of understanding only, and no unnecessary limitations should be understood therefrom, but the appended claims should be construed as broadly as permissible, in view of the prior art.

21 What I regard as new and desire to secure by Letters Patent is:

22 1. The method of forming a protective coating on the exterior surface of a surgical bandage consisting of a rolled fabric strip having plaster of Paris incorporated therein, which comprises preliminarily heating the bandage, dipping the heated bandage in a mixture of plaster of Paris and a boiling solution of a water-soluble adhesive material, and drying the dipped bandage while maintaining the same in heated condition.

23 2. The method of forming a protective coating on the exterior surface of a surgical bandage consisting of a rolled fabric strip having plaster of Paris incorporated therein, which comprises preliminarily heating the bandage to a temperature of about 98° centigrade, dipping the heated bandage in a mixture of plaster of Paris and a boiling solution of a water-soluble adhesive material, and drying the dipped bandage at a temperature not lower than 98° centigrade.

24 3. A surgical bandage comprising a roll of fabric impregnated with plaster of Paris and designed for immersion in water prior to use, and combined therewith a thin coating of water-permeable material applied thereon for preventing unrolling of the bandage and the escape of the plaster from the bandage prior to and during immersion, said permeable coating being resistant to disintegration during immersion to aid in maintaining the convolutions of the rolled bandage against telescoping during and after immersion incidental to its use, said coating permitting the penetration of water therethrough to the extent necessary to adequately moisten the plaster carried by the roll.

25 4. A surgical bandage comprising a roll of fabric having its convolutions impregnated with plaster of Paris in a dry comminuted state and designed for immersion in water prior to use, said roll having combined therewith means for preventing unwinding of the roll and the escape of plaster therefrom, said means consisting of a thin coating of water-permeable material applied to the exposed surfaces of the roll and being resistant to disintegration during immersion to aid in maintaining the convolutions of the rolled bandage against telescoping during and after immersion as an incident to the use of the bandage.

26 5. A surgical bandage comprising a roll of fabric incorporating plaster of Paris and designed for immersion in water prior to use, and combined therewith a thin coating of water-permeable material consisting of an adhesive, water-soluble gum applied to the surface of the roll for preventing unrolling of the latter and the escape of the plaster therefrom prior to and during immersion, said permeable coating being resistant to premature disintegration during immersion to aid in maintaining the convolutions of the rolled bandage against telescoping during and after immersion incidental to its use, said coating permitting the penetration of water therethrough to the extent necessary to adequately moisten the plaster carried by the roll.